

# UNITED STATES PATENT OFFICE.

JULIUS ASBECK, OF KRANTSHEID-WESTERWALD, GERMANY.

## PROCESS FOR OBTAINING REFINED LEAD.

1,025,956.

Specification of Letters Patent.

Patented May 14, 1912.

No Drawing.

Application filed May 20, 1910. Serial No. 562,377.

*To all whom it may concern:*

Be it known that I, JULIUS ASBECK, mining engineer, residing at Krantscheid-Westerwald, Germany, have invented certain new and useful Improvements in Processes for Obtaining Refined Lead, of which the following is a specification.

The object of the present process is to obtain pure lead in one single process out of lead-bearing material, and is especially intended for the treatment of old storage battery plates and the various waste material resulting from the manufacture and employment of lead accumulators.

Besides the greater simplicity of this process, it also has an advantage over all former processes in that it can be carried out in the melting pot at a low temperature.

The process consists in the heating of the lead-bearing material together with a mixture of caustic alkali and sulfur or sulfur containing compounds. It is probable that lead-sulfid is formed in the first stage, which in the second stage is reduced by the caustic alkali, at the same time forming sulfite or sulfate of the alkalis in question. The foreign metals present as compounds in the lead-bearing materials, are not reduced by this process, and the metallic impurities such as copper, antimony, arsenic and tin, are either oxidized or sulfurized, and enter into the dross or slag, so that perfectly pure lead is also obtained from impure working material.

An appropriate mixture consists of three parts of caustic soda to one part of sulfur, or equal parts of caustic soda and sodium thiosulfate, or three parts of caustic soda to one part of sulfid of sodium or sodium polysulfid. The lead-bearing materials are mixed with one of these mixtures and heated up to a temperature of 400-500° centigrade for a short time.

For further explanation it may be said that certain lead prior to treatment contained the following: copper .084%, nickel .0076% silver .008%. Five thousand pounds of such lead were employed along with thirty pounds of caustic soda (90% pure) and seventy pounds of sulfid of sodium (60% pure). The treatment was repeated three times and thereafter the lead contained copper .0072%, nickel .008% and silver .0081%. The proportions and results will vary somewhat and the presence or absence of dross in the lead to be treated will have its influence upon the number of times the treatment is to be repeated. However, from the foregoing illustration those skilled in the art will be able to obtain advantageous results by the practice of the invention.

I claim—

1. The process of refining lead which consists in adding a sulfid producing substance and caustic alkali thereto and mixing the ingredients in a molten condition and separating the lead from the slag.

2. The process of refining lead which consists in adding an alkaline sulfid and caustic alkali thereto and mixing the ingredients in a molten condition and separating the lead from the slag.

3. The process of refining lead which consists in adding sulfid of sodium and caustic soda thereto and mixing the ingredients in a molten condition and separating the lead from the slag.

In testimony whereof I affix my signature in presence of two witnesses.

JULIUS ASBECK.

Witnesses:

LOUIS VANDORY,  
BESSIE F. DUNLAP.